

E. A. PATERSON.

## BRIQUET COMPOSITION AND PROCESS OF MAKING BRIQUETS.

APPLICATION FILED DEC. 26, 1913.

1,111,919.

Patented Sept. 29, 1914.



### Witnesses

Alloprim  
E. B. Ferrioli

Inventor

Edward S. Paterson,  
of Baldwin Night  
his Attorney

# UNITED STATES PATENT OFFICE.

EDWARD ALFRED PATERSON, OF PORT ARTHUR, ONTARIO, CANADA.

## BRIQUET COMPOSITION AND PROCESS OF MAKING BRIQUETS.

1,111,919.

Specification of Letters Patent. Patented Sept. 29, 1914.

Application filed December 26, 1913. Serial No. 808,866.

*To all whom it may concern:*

Be it known that I, EDWARD A. PATERSON, a subject of the King of Great Britain, residing at Port Arthur, Province of Ontario, 5 and Dominion of Canada, have invented in certain new and useful Improvements in Briquet Compositions and Processes of Making Briquets, of which the following is a specification.

10 My invention relates to a method of and a composition for reassembling in any desired form suitable for the blast furnace, fine ore concentrates and dust containing silica, fine ore, iron ore flue dust, and the iron residues obtained from sulfuric acid works 15 wherein iron pyrites are roasted. Briquetting fine iron ore is done at the present time by various methods, but these methods require expensive machinery, and the cost of operation 20 is heavy. I have found it advisable to treat the ore in the following way, which is economical and puts the material in good condition for the furnace.

Briquets, as heretofore made, have been 25 usually hard and smooth, and frequently do not offer sufficient points for attack by the heat, but in some cases this form of the material is preferred, as some furnace men, being accustomed to some particular shape desire to have the material compressed into 30 briquets of that shape. Mine are preferably somewhat irregular in shape, or lumpy.

The accompanying drawing shows an apparatus by means of which my process may 35 be effectively carried out.

Figure 1 shows a general view of the apparatus partly in side elevation and partly in section and with some of the parts broken away. Fig. 2 is a detail view in perspective 40 of the mold faced roll employed.

1 indicates an ordinary mixing machine, such as a concrete mixer, into the hopper 2 of which the fine ore, water and silicate are put. These, when mixed, are discharged 45 upon a belt 3, which may be an endless steel band or of some other material heavy enough to carry the ore and sufficiently resistant to the heat. At 4, I have shown a corrugated or mold-faced roll. Opposed to this is a roll 50 5. Between these the belt laden with the wet ore mass is carried and the mass is broken or cut up or molded by the mold-shaped roll into more or less uniformly sized

rough masses or lumps, without much pressure.

Just before the mass is discharged upon the belt, at 6, I distribute upon the belt a layer of ore dust discharged down the chute 7 from a bin or hopper 8. This ore dust prevents the lumps or masses of ore from sticking to the belt, and itself adhering to the lumps, gives them a rough surface, yielding readily to the smelting action. Below the upper course of this belt I have indicated a heater 9, i. e. a gas pipe with a number of burners, though, of course, other heating means may be used. This belt should be long enough and should move at such speed that the briquets or lumps are dry enough to be hard when they are finally discharged at 10, passing from the belt to the discharging point down chute 11. The upper part of this chute is perforated or reticulated at 11', so that any unattached ore dust will fall off and be discharged into a box 12, whence it 15 may be lifted by conveyer 13 to hopper 8. In said hopper 8 I provide a stirrer 14. A shaking table 15 may be used, discharging through tube or funnel 16 at or near the exit opening of the hopper.

It will be noted that by drying the lumps or briquets before they are removed from the belt, I avoid the danger of their breaking or crumbling.

The fine ore is mixed with the calculated 85 amount of flux, and to this is added ten to fifteen per cent. of water, if the material is dry, and from five to ten per cent. of silicate of soda solution of 50° Twaddell. After the materials have been well mixed, the charge 90 is fed onto the traveling belt which is heated to from 120 to 150 degrees C., the length of the belt being so adjusted that the material is, from fifteen to twenty minutes exposed to the heat. The thickness of the material 95 must, of course, be adjusted to give a hard and compact product after it leaves the belt. The silicate of soda dries and the particles cohere together.

I have found it advisable and economical 10 to introduce into each briquet some base for the silicic acid in quantity just about enough to take care of all the silica in the ore. This base, ordinarily would be lime preferably in the form of limestone which 10 is the cheapest. Lime itself is not a very

good agglomerant. I find it useful to use an alkaline silicate as an agglomerant or binder. The silicate which I prefer to use is a hydrous silicate of sodium which has, as compared with other alkali silicates, usually available, a larger proportion of silicic acid. The formation of this is typified by the formula



The equivalent of  $n$  is anywhere from two to four and the value of  $x$  is two or three. To this silicate, when mixed with water, I add pulverized limestone. With this mixture I then briquet the ore by molding or lumping in the manner indicated. The briquets may be exposed to the atmosphere, and it will be found that in time they acquire a hard surface and this condition may penetrate throughout the mass. I attribute this hardening to the effect of carbonic acid in the atmosphere which goes to the sodium base of the silicate forming sodium carbonate and freeing the hydro-silicic acid, which thus becomes the effective binder of the briquet. The calcium carbonate remains unchanged at the end of the reaction and I attribute to this carbonate a catalytic effect during the progress of the change. That is, I am of the opinion that the calcium carbonate passes one molecule of  $\text{CO}_2$  over to the soda, and takes another molecule of  $\text{CO}_2$  from the air, and that it will keep this up until all the soda changes to carbonate, or until the mass becomes too dry for the reaction to occur. Without the catalytic agent the action of the  $\text{CO}_2$  upon the sodium component of the silicate is much slower.

Briquets thus made can be smelted in an ordinary manner, and during the smelting the soda will mainly be volatilized. Enough limestone must be added to take care of the additional silicic acid, which is not changed, used in the binder. If it is desired to lump the material without the flux, I treat it mechanically in the presence of  $\text{CO}_2$  in the same way indicated above, but I only use from four to six per cent. of the silicate solution and the same quantity of water. I simply add the water so as to get the materials well mixed together, and as the water has to be evaporated later, I merely use enough to make the mixture into a somewhat stiff plastic condition. If I use five per cent. of the silicate solution of the above indicated strength, the amount of real silicate is about one per cent., and if I use the hydrous silicate I make allowance for the combined water; and on the other hand, I add more water if the hydrous silicate be mixed with the other materials before the water was added in the mixer, that is, instead of ten to fifteen per cent. water I use fifteen to twenty-five per cent.

The following proportions are suggested. Much depends upon the character of the ore: fine iron ore 100 grams, water 15 c.c., silicate of soda 4 c.c. of  $50^\circ \text{ T}$ . With the flux added these proportions may be used: fine iron ore 77 grams, water 15 c.c., limestone 33 grams, silicate 10 c.c.

In the smelting operation the small amount of alkali undoubtedly aids the lime somewhat in fluxing the silica, but probably before the smelting operation is complete, as indicated above, most of this alkali disappears through volatilization.

I claim as my invention:

1. The process of briquetting a silicious ore, which consists in mixing with a hydrous alkali silicate an alkali earth carbonate, and agglomerating said ore with said mixture. 80

2. The process of briquetting a silicious ore, which consists in mixing with an alkali silicate, a hydrous alkali earth carbonate, and agglomerating said ore with said mixture, the quantity of alkali earth carbonate being proportioned to the total quantity of silicic acid in the agglomerated briquet. 85

3. The process of briquetting silicious iron ore, which consists in mixing with hydrous sodium silicate pulverized limestone and briquetting said ore with said mixture. 90

4. The process of briquetting silicious ore, 95 which consists in mixing with hydrous sodium silicate an alkali earth carbonate, agglomerating said ore with said mixture, the quantity of said carbonate being proportioned to the total quantity of the silicic acid in the finished briquets, and exposing them to the hardening effect of carbon dioxid. 100

5. A process for briquetting or lumping ore dust, which consists in mixing said ore 105 dust with a hydrous alkali silicate, in solution, and water, discharging upon a suitable surface a layer of powdered ore, discharging upon said layer the mixed ore and silicate, molding or lumping said mixture upon said surface, drying the lumps so formed upon the same surface, discharging the said lumps from said surface, and at the same time separating from said lumps any unattached powdered ore. 110

6. A process for briquetting or lumping fine ore, which consists in mixing to a stiff plastic condition said ore with hydrous alkali silicate, in solution, water and pulverized limestone, discharging upon a suitable moving surface a layer of powdered ore, discharging upon said layer the mixture of ore, water, silicate and limestone, molding or lumping it upon said surface, causing the lumps so formed to pass undisturbed upon said surface through a drying zone until the lumps become hard, and then passing the lumps off said surface and at the same time separating from said lumps any unattached ore. 115 120 125

7. A process for briquetting or lumping ore dust, which consists in mixing said ore dust with hydrous alkali silicate, in solution, and water, discharging upon a suitable surface a layer of powdered ore, discharging upon said layer the mixed ore and silicate, molding or lumping said mixture upon said surface, drying the lumps so formed upon the same surface, discharging the said lumps from said surface, and at the same time separating from said lumps any unattached powdered ore, and finally exposing said lumps to the hardening effect of carbon dioxide.
- 10 8. A composition for briquetting pulverized ore, which consists of a mixture of a hydrous alkali silicate and an alkali earth carbonate.
9. A composition for briquetting pulverized ore, which consists of hydrous sodium silicate and limestone pulverized, the quantity of limestone being proportioned to the total quantity of silica in the silicate and in the ore.
- 15 In testimony whereof, I have hereunto subscribed my name.

EDWARD ALFRED PATERSON.

Witnesses:

LEWIS T. PAYNE,  
ELSIE SCHMITT.